

May 25, 1948.

D. F. DRIESCHMAN

2,442,163

CATHODE STRUCTURE

Original Filed Aug. 31, 1943 2 Sheets-Sheet 1



INVENTOR.  
Donald F. Drieschman  
BY *Harold E. Long*

HIS ATTORNEY

May 25, 1948.

D. F. DRIESCHMAN

2,442,163

CATHODE STRUCTURE

Original Filed Aug. 31, 1943 2 Sheets-Sheet 2



Fig 4



Fig 5

INVENTOR.  
Donald F. Drieschman  
BY *Harold E. Long*

HIS ATTORNEY

## UNITED STATES PATENT OFFICE

2,442,163

## CATHODE STRUCTURE

Donald F. Drieschman, San Carlos, Calif., assignor to Eitel-McCullough, Inc., San Bruno, Calif., a corporation of California

Original application August 31, 1943, Serial No. 500,717. Divided and this application September 1, 1944, Serial No. 552,310

4 Claims. (Cl. 250—27.5)

1

This is a division of my copending application, Serial No. 500,717, filed August 31, 1943, now abandoned.

My invention relates to a cathode structure for electron tubes.

It is among the objects of my invention to provide a filamentary type cathode embodying an improved welded joint between the filament wires and their supports.

Another object is to provide an improved method of fabricating a cathode structure of the character described.

The invention possesses other objects and features of advantage, some of which, with the foregoing, will be set forth in the following description of my invention. It is to be understood that I do not limit myself to this disclosure of species of my invention as I may adopt variant embodiments thereof within the scope of the claims.

Referring to the drawings:

Figure 1 is an elevational view of a cathode structure embodying the improvements of my invention; and

Figure 2 is an enlarged detail sectional view taken in a plane indicated by line 2—2 of Figure 1, showing the welded joint and special alloy formed at the weld.

Figure 3 is an exploded vertical sectional view of the cathode and assembly jig.

Figure 4 is a vertical sectional view of a cathode in a bell jar ready for arc welding.

Figure 5 is a plan view of a modified arrangement for welding, using a high frequency coil.

In terms of broad inclusion, my cathode structure comprises a plurality of filament wires welded at opposite ends to metallic supports by a metallic welding material. The material used to make the weld comprises a refractory metal, such as columbium or tantalum, and preferably includes a minor proportion of another metal, such as ruthenium. One of the supports is movable, and means associated with the movable support is provided for tensioning the filament wires. An improved method is also provided for holding the filament wires and supports in assembled relation during the welding operation.

In greater detail, and referring to the drawings, my improvements are illustrated in conjunction with an electrode for a vacuum tube, and more particularly to a cathode structure. As shown in Figures 1 and 2, the cathode comprises a multiplicity of say 40 parallel wires 2 of thoriated tungsten divided into four groups disposed in cylindrical formation about the cathode axis, each group of wires being connected at the lower

2

end to one of the four tungsten cathode leads 3 and all being connected at the upper end to a common terminal 4.

Fixed supports for the lower ends of the filament wires are provided by brackets 6 welded to the leads and to quadrant sections 7 having arcuate rims to which the groups of filament wires are welded. Leads 3 are sealed in a four-way press 8 on a suitable stem 9 of glass or the like. The upper support or terminal 4 is a cap having a circular rim to which the upper ends of the filament wires are welded. These upper and lower supports are of a refractory metal such as tantalum or molybdenum, tantalum being preferred.

Top cap 4 provides a movable support and is held centered by a tungsten rod or standard 11 sealed to the stem and projecting through the cap. Tension is uniformly applied to all the filament wires by a sleeve 12 slidable along the center rod and urged upwardly against cap 4 by a spring 13 interposed between the sleeve and stem.

In the final tube diametrically opposed cathode leads 3 are connected in parallel to a source of heating current. Since two of the groups of filament wires are connected in series with one pair of leads and the other two groups are connected in series with the other two leads, all of the filament wires are simultaneously heated. This structure has the advantage of compacting a multiplicity of filament wires in a relatively small circle, whereby a large amount of electron emitting surface is made available.

The main problem in fabricating such a structure is of course securing the ends of the filament wires to the supporting members. Ordinary spot welding practice is not feasible because of the close spacing between the wires. I have solved the problem by a special material and welding technique, resulting in the formation of a bonding medium or layer 14 in which the filaments are embedded. See Figure 2. This layer preferably comprises an alloy composed of a major proportion of columbium and a minor proportion of ruthenium, the preferred proportions being about 4% to 20% by weight of ruthenium and the balance columbium. Other refractory metals such as tantalum may be substituted in whole or in part for the columbium component of the alloy. Likewise other metals in group 8 of the periodic table may be substituted for the ruthenium component. However the columbium-ruthenium composition is superior in many respects and is preferred. This alloy has a high melting point, low vapor pressure, is very hard and makes an

excellent bond between refractory metals such as tungsten and the like. These properties make the alloy especially suited for a joint structure in a cathode where exceedingly high temperatures are involved.

The preferred method of making the cathode utilizes a jig (Figure 3) comprising a cylindrical core 16 of say copper having longitudinal grooves in the surface to receive filament wires 2, the latter being straight, rod-like pieces cut to size. These wires are temporarily held by a rubber band 17; core 16 being proportioned so that wires 2 project freely from the ends. At this stage of fabrication the quadrant sections on brackets 6 are formed as a one-piece ring 18 which is later severed at four places to make the individual quadrants. Ring 18 is inserted at the lower end of the jig-held filament wires and top cap 4 is inserted at the upper end, the jig core being sized to hold wires 2 in a circle slightly smaller in diameter than that of the end supports so that the latter are held by press fit during the welding operation. As shown in Figure 4, a handle 19 is threaded into core 16 to permit moving the assembled cathode up into a bell jar 20 for welding purposes.

The material used to produce the preferred bonding alloy at the weld comprises a mixture of finely divided particles of columbium and ruthenium. The columbium particles should not be larger than about 200 mesh, a particle size of around 400 mesh being preferred. The ruthenium particles used are preferably still more finely divided, a powder known commercially as "ruthenium black" being preferred. These particles are mixed together with a liquid vehicle, such as water, to a thin pasty consistency suitable for application with a brush. This material is then brushed onto the rims of the supports and over the end portions of the filament wires as shown at 15 in Figure 4.

With the material applied the assembled cathode is then elevated in bell jar 20 to position the upper support near an electric arc discharging between electrodes 21 sealed to the sides of the bell jar. Rotation of the cathode by the operator exposes successive portions of the rim to the intense heat of the arc. After finishing the top weld the structure is moved up to weld the filaments at the lower support. A non-oxidizing atmosphere is maintained in the bell jar by admitting a gas, such as hydrogen, through a suitable duct 22.

In making these welds I find that the material melts and flows out uniformly and smoothly over the joint. The ruthenium performs an important function at this stage, serving as a wetting agent and to give uniform spreading of the material over the surfaces. The final composition formed by the columbium and ruthenium is a hard, 60 tough alloy having good bonding affinity for other refractory metals such as the tungsten filaments 2 and tantalum supports 4 and 18. These properties insure strong mechanical joints at the ends of the filaments. Furthermore the high melting point and low vapor pressure of the bonding medium produces a weld which will readily withstand the incandescent operating temperatures of the filament wires.

Instead of using an arc the heat required for 70 making the weld may be supplied by high frequency induction, using a coil 23 as shown in

Figure 5; this coil being positioned in a suitable bell jar so that the non-oxidizing atmosphere may be supplied. The assembled cathode on the jig is elevated to place the desired portions of

- 5 the cathode within the coil, whereupon the coil is energized to induce the required amount of heat. Since lower support 18 is a continuous ring at this time the induction heating method may be used at the bottom as well as at the top welds. 10 After the welds are completed ring 18 of the lower support is cut in four places between brackets 6 to separate it into the quadrant sections 7 shown in Figure 1. Jig core 16 is then removed by spreading the lower end of the cathode. The 15 cathode is now ready for final mounting, together with the spring tensioning device, on stem 9.

I claim:

1. A cathode structure comprising spaced supports of refractory metal, tungsten filament wires secured to said supports by a metallic welding material, the metal of said material consisting essentially of an alloy of columbium with from 4% to 20% of ruthenium. 20 2. A cathode structure comprising spaced supports of refractory metal, and tungsten filament wires secured to said supports by a metallic welding material, the metal of said material consisting essentially of an alloy of refractory metal selected from the group consisting of columbium and tantalum with a minor proportion of ruthenium. 30 3. A cathode structure comprising spaced supports of refractory metal, and tungsten filament wires secured to said supports by a metallic welding material, the metal of said material consisting essentially of an alloy of refractory metal selected from the group consisting of columbium and tantalum with from 4% to 20% of ruthenium. 35 4. An electrode structure comprising members of refractory metal secured together by a metallic welding material, the metal of said material consisting essentially of an alloy of a refractory metal selected from the group consisting of columbium and tantalum with a minor proportion of ruthenium. 45

DONALD F. DRIESCHMAN.

#### REFERENCES CITED

The following references are of record in the file of this patent:

#### UNITED STATES PATENTS

| Number     | Name             | Date          |
|------------|------------------|---------------|
| Re. 13,961 | Zimmerman        | Aug. 10, 1915 |
| 991,578    | Whitney          | May 9, 1911   |
| 1,115,426  | Liebman          | Oct. 5, 1915  |
| 1,389,351  | Harvey           | Aug. 30, 1921 |
| 1,730,003  | Goldsmith et al. | Oct. 1, 1929  |
| 1,807,885  | Weingartner      | June 2, 1931  |
| 2,072,676  | Jedele           | Mar. 2, 1937  |
| 2,075,639  | Castle           | Mar. 30, 1937 |
| 2,097,178  | de Golyer        | Oct. 26, 1937 |
| 2,188,636  | Vilensky         | Jan. 30, 1946 |
| 2,225,853  | Baker            | Dec. 24, 1940 |
| 2,298,929  | Dailey           | Oct. 13, 1942 |
| 2,341,716  | Herdman          | Feb. 15, 1944 |
| 2,350,270  | Atlee            | May 3, 1944   |

#### FOREIGN PATENTS

| Number  | Country | Date         |
|---------|---------|--------------|
| 528,688 | Germany | July 2, 1931 |